

1

3,694,207

**TREATMENT OF IMAGEWISE EXPOSED CATALASE ACTIVE OR PEROXIDASE ACTIVE ENZYME CONTAINING LAYER WITH PEROXIDE**

Reinhart Matejec and Erwin Ranz, Leverkusen, Germany, assignors to Agfa-Gevaert Aktiengesellschaft, Leverkusen, Germany

No Drawing. Filed Oct. 26, 1970, Ser. No. 84,195  
Claims priority, application Germany, Nov. 6, 1969,

P 19 55 901.4  
Int. Cl. G03c 5/24

U.S. Cl. 96—48

6 Claims

**ABSTRACT OF THE DISCLOSURE**

For the production of positive photographic images are used layers containing catalase active and/or peroxidase active enzymes, which are inactivated on exposure to light, thus becoming incapable of decomposing peroxide compounds. The peroxide compounds are used either to form an image of gas bubbles in the layer or to produce a dye image by a color-forming oxidation reaction. The sensitivity can largely be increased by substances which on exposure to light liberate halogen or cyanide, which latter products act as poisons for the enzymes.

The invention relates to a process for the production of photographic images by the imagewise inactivation of catalase active and/or peroxidase active enzymes by the exposure of a light-sensitive layer and the imagewise decomposition of peroxide compounds by these enzymes, a visible image being formed by the imagewise production of gas bubbles either by physical means or by an imagewise color-forming reaction of the resulting oxygen with a suitable reactant.

Apart from the conventional photographic processes which make use of light-sensitive silver halide emulsion layers, numerous other processes have already become known for the production of photographic images. Thus, for example, bubble images can be produced by means of a photographic material comprising a layer which contains, dispersed in a binder, a compound which can be decomposed by light, e.g. a diazo salt. When such a material is exposed to form an image, the compound decomposes in areas corresponding to the image, a gas being liberated in the process. The gas bubbles expand as a result of the subsequent heating of the exposed material, and a bubble image is formed. Since the bubbles formed scatter the light imagewise, these areas appear dark in transmitted light and bright in reflected light. Most of the incident light in the unexposed areas of the layer is transmitted.

Belgian Pat. No. 725,903 also discloses the production of photographic images which consist of a silver image and a bubble image superimposed on the silver image. According to the process described there, a silver image is first produced in the conventional way in a hydrophilic layer, but this image has substantially less covering power than the conventionally produced black and white images. The layer is then brought into contact with hydrogen peroxide which decomposes imagewise in the areas containing the silver in a finely divided form to yield oxygen bubbles. The silver image is thus greatly intensified and deep black images with high contrast are obtained even when layers which have a very low silver content are used. Although the quality of the photographic images obtained by this process is satisfactory, the process is disadvantageous in that a silver image must first be produced by the usual conventional development, and this silver image is then reacted in a second stage

2

with hydrogen peroxide so as to produce the bubble image which is superimposed on the silver image. The process is, therefore, rather complicated. Moreover, only negative images of the original can be obtained directly by this process.

The other known photographic processes which do not use silver halide layers are, generally speaking, of only slight practical importance owing to their low sensitivity to light. The reason for this is that in contrast to conventional silver halide photography, the quantum yield is low in these light sensitive systems since per absorbed light quantum only one molecule can be converted photochemically with color-forming. No multiplying effect occurs as in the development of conventionally exposed silver halide emulsion layers.

It is an object of the invention to evolve photographic direct positive production processes as far as possible free from silver which result in black and white or colored images with sufficient contrast by a simple processing technique.

A process for the production of positive photographic images by imagewise exposure of a layer followed by treatment with a peroxide compound with formation of a visible image has now been found in which a light-sensitive layer is used which contains uniformly distributed catalase active or peroxidase active enzymes which are inactivated imagewise by exposure with actinic light.

Practically any light-sensitive enzymes are suitable for the process according to the invention, i.e. enzymes which are inactivated by the action of light and which are capable of catalytic decomposition of peroxide compounds. Examples of such enzymes are catalase, peroxidase, haemoglobin and haematin.

The sensitivity of the layers to light can be substantially increased by the addition of compounds which, when exposed to light, split off products in areas corresponding to the image which act as poisons for the enzymes used according to the invention, i.e. such added compounds have an additional inactivation effect on these enzymes in the exposed areas. Since the catalase active or peroxidase active enzymes used according to the invention generally contain iron, bound in the form of a complex, the substances most suitable for this purpose are inorganic or organic substances liberating halogen or cyanide on exposure to light, which products are capable of inactivating these enzymes.

Suitable inorganic halides which split off halogen on exposure to light are, for example, silver halides such as silver chloride, silver bromide or silver iodide. Suitable organic halides include aliphatic halides containing a tribromo or triiodo group, e.g. iodoform, tribromoethanol or tribromoacetic acid or highly halogenated aromatic compounds, e.g. benzenes which are substituted in at least three positions on the nucleus with bromide or iodine, e.g. pentabromophenol. Compounds of this type have been described e.g. in British Pat. No. 957,192.

Inorganic and organic cyanide compounds which split off cyanide on exposure to light include in particular iron-(II) cyanides or iron-(III) cyanides or complex cyanides or complex cyanides or nitro-prussides described e.g. in the book by M. H. Ford-Smith "The Chemistry of Complex Cyanides," London, 1964. Suitable organic compounds include cyanides of triphenylmethane and its derivatives, e.g. those described by A. H. Spore, Trans. Faraday Soc. 57 (1961), 983.

The sensitivity can also be increased by the addition of compounds which generally act as electron acceptors. Chloranil or tetracyano-p-quinodimethane, for example, are suitable.

The light used for exposure is preferably blue or ultraviolet light.

The images obtained on exposure are practically invisible. They are brought into contact with peroxide compounds, such as hydrogen peroxide, to render them visible. The peroxide compound is decomposed imagewise in the areas where the enzymes have remained active. The process of rendering the image visible by decomposition of the peroxide may be either physical or chemical. For example, the oxygen evolved can be rendered visible as a bubble image, e.g. by the process described in the above-mentioned Belgian Pat. No. 725,903 which corresponds to U.S. Ser. No. 783,420. It is also possible to decompose the peroxide compounds in the presence of reactants for a color-forming oxidation reaction. Such processes are described in U.S. application Ser. No. 881,610.

The layers according to the invention preferably contain the light-sensitive enzymes, e.g. catalase or peroxidase, dispersed in a binder. Suitable binders are e.g. silica gel, polyvinyl acetate, partly saponified polyvinyl acetate, polyvinyl alcohol, cellulose esters such as cellulose acetate or cellulose butyrate, carboxymethyl cellulose or natural binders, especially proteins such as gelatin.

On the other hand, the enzymes may be added directly to the layer support by treating the support with a solution or dispersion of the enzyme.

The concentration of the enzymes in the light-sensitive material may vary within wide limits. Concentrations of between 0.3 and 5 g./m.<sup>2</sup> of light-sensitive material have been found to be suitable. The optimum quantity for any given reproduction process can be determined by a few simple laboratory tests.

Nearly the same applies to the quantity of additives used for increasing the sensitivity of the layers. Their concentration may also vary within wide limits. Quantities of between 0.2 and 5 g./m.<sup>2</sup> have been found sufficient in this case, depending on the nature of the light-sensitive compounds. The optimum concentrations and optimum pair of compounds consisting of the enzyme and the substance which increases the sensitivity can easily be determined by the usual tests.

Suitable peroxide compounds for the process according to the invention are inorganic peroxide compounds, e.g. perborates, percarbonates or persulfates, but especially hydrogen peroxide. Organic peroxide compounds, e.g. benzoyl peroxide, are also suitable. Hydrogen peroxide is used for preference owing to its efficiency and the ease with which it can be handled in the form of aqueous solutions.

The peroxide compound is preferably applied in the form of a solution. Hydrogen peroxide, for example, may also be applied in vapor form.

For the production of a bubble image, the exposed layer is heated with hydrogen peroxide during or after the treatment. A bubble image then forms imagewise in the areas where the enzymes have remained active.

The strength of the bubble image depends on the quantity of hydrogen peroxide used and on the quantity of decomposition nuclei formed. The heat treatment of the material for producing the visible bubbles should be as short as possible. The temperature to be maintained during this treatment depends on the properties of the binder. Satisfactory results can already be obtained at relatively low temperatures of about 60° C. to 70° C. but higher temperatures may also be employed if the softening point of the binder requires this. If the binder used is gelatin, which is the substance preferably used, it is advisable to work in the presence of small quantities of water because this promotes swelling of the gelatin and hence the formation of bubbles. The same applies to other binders which swell in water.

According to a preferred embodiment, after the layer has been exposed to light and treated with hydrogen peroxide vapor, it is exposed for a few seconds, e.g. 1.5 seconds, to a water vapor atmosphere of about from 50° C. to 90° C. The formation of bubbles, which sets in only slowly when using hydrogen peroxide alone, then starts

very quickly. It has been found even more advantageous to expose the layer, after treatment with the hydrogen peroxide, to an alkaline water vapor atmosphere at pH values of between 8 and 12. This can easily be achieved by adding small quantities of ammonia or vapors of volatile amines to the water vapor. The concentration of the alkaline additives in the vapor is not critical. Quantities of between 0.1 and 5 volumes percent, preferably about 0.3 to 1 volume percent have generally been found sufficient.

The use of peroxides mixed with hydrazines has also been found very advantageous for the catalytic production of the bubble image; not only O<sub>2</sub> but a mixture of O<sub>2</sub> and N<sub>2</sub> is then formed.

The bubble images obtained can be stabilized against moisture by the processes described in U.S. application Ser. No. 885,984 and Ser. No. 887,392 as required.

The visible image may also be produced chemically by carrying out the treatment of the exposed layer with the peroxide compound in the presence of reactants for a color-forming oxidation reaction. Suitable processes have been described in U.S. application Ser. No. 881,610.

Especially suitable for the oxidative color-formation are, of course, those reactants which produce very deeply colored compounds on oxidation with the catalytically activated peroxide compound.

These reactants may be organic compounds which themselves yield the image dye on oxidation, e.g. amino, hydroxy or aminohydroxy compounds of isocyclic or heterocyclic aromatic compounds.

The following are mentioned as examples:

phenol,  
aniline,  
pyrocatechol,  
35 resorcinol,  
hydroquinone,  
o-, m- and p-phenylenediamine,  
N,N-dimethyl-phenylenediamine,  
N,N-diethylphenylenediamine,  
40 N-ethyl-N-methyl-phenylene diamine,  
o-, m- and p-aminophenol,  
p-methylaminophenol,  
2,4-diaminophenol-(1),  
1,7-dihydroxynaphthalene,  
2,3-dihydroxynaphthalene,  
45 1,6,7-trihydroxynaphthalene,  
1,2-diaminonaphthalene,  
1,8-diaminonaphthalene,  
benzidine,  
2,2'-diaminodiphenyl,  
4,4'-diaminodiphenyl,  
8-hydroxyquinoline,  
5-hydroxyquinoline,  
2-hydroxycarbazole and 1-phenylpyrazolone-(3)

The amino, hydroxy or aminohydroxy compounds may also be substituted, e.g. with halogen, alkyl, aryl, alkoxy, sulfonic acid, nitro acyl, carboxylic acid or carbonamide groups. The following are mentioned as examples:

60 2,5-dichloro-p-phenylene diamine,  
guaiacol,  
4-methoxynaphthol-(1)  
1-hydroxy-2-aminobenzene-4-sulfonic acid,  
1-amino-2-hydroxybenzene-4-sulfonic acid,  
3-amino-5-sulfo-salicylic acid,  
65 1,6,7-trihydroxynaphthalene-3-sulfonic acid,  
benzidine-2,2'-disulfonic acid,  
benzidine-3,3'-disulfonic acid,  
1,8-dihydroxy-naphthalene-disulfonic acid-(3,6) and  
4-nitro-pyrocatechol.

In some cases, mixtures of several such compounds result in a much stronger dye formation on oxidation than the individual components. Thus, for example a mixture of o-phenylene diamine and pyrocatechol yields stronger dye formation. Even components which on their

## 5

own do not yield dyes on oxidation, e.g. tetrabromo-  
hydroquinone or tetrabromopyrocatechol, are capable of  
increasing dye formation when added to other hydroxy,  
amino or aminohydroxy compounds.

Oxidation of the aromatic amino, hydroxy and/or  
amino hydroxy compounds yields monomeric or poly-  
meric dyes which are related to quinone imines and  
azines. Some examples of these oxidative dye formations  
are described in "Künstliche organische Farbstoffe und  
ihre Zwischenprodukte" by H. R. Schweizer, Springer-  
Verlag, Berlin-Göttingen-Heidelberg (1964), pages 222,  
275, 281 and 293; in "Grundlagen der Synthese von  
Zwischenprodukten und Farbstoffen," by N. I. Woro-  
show; Akademie-Verlag, Berlin (1966) pages 703 to 789;  
in "Chemie der Farbstoffe und deren Anwendung" by A.  
Schaeffer, (Technische Fortschrittsberichte, volume 60),  
Theodor-Steinkopff-Verlag, Dresden-Leipzig (1963), pages  
59 et seq.

In addition to dye precursor compounds there may,  
of course, also be used leuco dye compounds and vat  
dyes which are capable of being oxidized to dyes. For  
example of these see "Künstliche organische Farbstoffe  
und Zwischenprodukte," by H. R. Schweizer, Springer-  
Verlag, Berlin-Göttingen-Heidelberg (1964), pages 250  
and 320.

Also suitable for the process according to the invention  
are those organic compounds capable of oxidation  
which yield the image dye only in a secondary reaction  
with other compounds. In principle, any reaction sys-  
tems which yield dyes by oxidative coupling may be used,  
in particular the so-called color-forming photographic  
developers of the phenylenediamine or aminopyrazolone  
series (see e.g. C. E. K. Mees and T. H. James: "The  
Theory of the Photographic Process," 3rd edition, Mac-  
Millan Co., New York (1966), page 382; H. R. Schweizer;  
Künstliche organische Farbstoffe und ihre Zwischen-  
produkte," Springer-Verlag, Berlin-Göttingen-Heidelberg  
(1964), page 295). Isoyclic and heterocyclic hydrazines  
may also be coupled with suitable components to yield  
dyes by oxidation (see e.g. H. Hünig et al., Angewandte  
Chemie 70 (1958); S. Hünig, Chimia 15 (1961) 133  
and Angewandte Chemie 74 (1962) 818). The color-  
forming photographic developer substances are catalytically  
oxidized by the peroxide compounds at the image-  
wise distributed catalyst. Their oxidation products may  
then react with known photographic color-forming cou-  
plers present at the same time to form dyes. Suitable  
color-forming couplers for this purpose are, for ex-  
ample, those of the phenol or naphthol series as cyan-  
forming couplers, those of the indazolone and pyrazolone  
series as magenta-forming couplers and those of the  
benzoyl acetanilide series as yellow-forming couplers.

The following examples illustrate the invention:

## EXAMPLE 1

100 ml. of an aqueous 10% solution of a ferri-tri-  
bromoacetate complex compound (to split off halogen;  
prepared by suspending excess  $Fe(OH)_3$  in 10% sodium  
tribromoacetate solution  $CBr_3-COONa$  and filtering from  
the excess  $Fe(OH)_3$ ) are added in the dark to 1 l. of  
a 5% aqueous carboxymethyl cellulose solution. 100 ml.  
of a 0.1% aqueous peroxidase solution are then added.

The mixture is then poured in a thin layer onto a  
layer support of paper. It is then hardened by bathing it  
for one minute in 1%  $Ba(NO_3)_2$  solution and dried.

The layer is exposed to blue light behind a grey step  
wedge (exposure time with a 200 watt lamp 10 seconds).  
It is then treated with the following solution:

20 g. of 1,7-dihydroxynaphthalene <sup>1</sup>  
40 g. of phenylhydrazine sulfonic acid-(2) <sup>1</sup>  
Water up to 1 l.; adjusted to pH 11 with  $Na_2CO_3$   
5 ml. of 30% aqueous  $H_2O_2$  added just before use

## 6

A black and white positive dye image of the original  
is obtained within 5 minutes.

Finally, the layer is washed for 15 minutes and dried.

## EXAMPLE 2

20 ml. of a dispersion which contains 100 g. of silver  
bromide and 20 g. of carboxymethylcellulose per liter  
are added as light-sensitive halogen donor to 1 l. of an  
aqueous 2% carboxymethylcellulose solution in the dark.  
100 ml. of an alkaline 1% aqueous haemoglobin solution  
are then added as peroxidase active catalyst. The  
mixture is poured out in a thin layer on a cellulose  
acetate support. It is then hardened as described in Ex-  
ample 1 and dried.

The layer is exposed to white light behind a grey step  
wedge (exposure time with a 200 watt lamp 1 second)  
and then treated with the following solution:

25 g. of 1-aminonaphthol-8-sulfonic acid-(4) <sup>1</sup>  
10 g. of 2-ethoxyphenol <sup>1</sup>  
Made up to 1 l. with water, adjusted to pH 8 with  $Na_2CO_3$   
100 ml. of 30% aqueous  $H_2O_2$  added just before use.

<sup>1</sup> As dye forming reactants.

25 A black and white positive dye image of the original  
is obtained within 5 minutes at 20° C. Lastly, the layer  
is washed for 15 minutes and dried.

## EXAMPLE 3

30 50 g. of tribromoethanol as halogen donor are dis-  
solved in 2 l. of an aqueous 6% gelatin solution in the  
dark. 25 ml. of a 0.1% catalase solution are then added  
to the above solution. The mixture is then poured out  
35 as a thin layer on a layer support of polyethylene ter-  
ephthalate (layer thickness approximately 15 $\mu$ ).

It is exposed in a sensitometer behind a grey step  
wedge as described in Example 1. The exposed material  
is then subjected to a water vapor atmosphere at about  
40 50° C. for about 1/2 second.

For bubble formation, the layer is treated for about  
30 seconds with saturated hydrogen peroxide vapor at  
70° C. and then exposed for 1/2 second to a water vapor  
atmosphere at 75° C.

45 An image which has a density of 1.8 in collimated  
white light is obtained.

## EXAMPLE 4

50 25 ml. of a 1% catalase solution are added to 1 l. of  
a 6% gelatin solution. 50 ml. of a saturated solution  
of Malachite green leucocyanide (nitrile of Malachite  
green; substance which splits off cyanide) are then emul-  
sified in ethyl acetate in the dark with vigorous mixing.  
The solution is then cast and the material is processed  
55 to produce a bubble image, as described in Example 3.

We claim:

1. In a process for the production of positive photo-  
graphic images by imagewise exposure of a light-sensitive  
60 layer, the steps of imagewise exposure of a light-sensitive  
layer containing uniformly distributed in a binding agent  
a catalase active or peroxidase active enzyme, which  
enzymes are capable of decomposing peroxide compounds  
and capable of being inactivated by exposure to actinic  
light, and treating the exposed layer with a peroxide  
compound.

2. In the process of claim 1 the light-sensitive layer  
contains compounds which split off halogen or cyanide  
on exposure to light.

3. In the process according to claim 1, the enzyme and  
peroxide is contained in a binder selected from the group  
70 consisting of gelatin, silica gel, polyvinyl acetate, partly  
saponified polyvinyl acetate, polyvinyl alcohol, and  
cellulose esters in which binder the peroxide is decom-  
posed.

<sup>1</sup> As dye forming reactants.

4. In the steps of the process according to claim 1, mixtures of peroxide compounds are used.

5. In the steps of the process according to claim 1, producing a color-forming oxidation reaction by treating the exposed layer with peroxide compounds in the presence of a reagent selected from the group consisting of amino-, hydroxy-, and amino-hydroxy isocyclic aromatic compounds and amino-, hydroxy- and amino-hydroxy heterocyclic aromatic compounds. 5

6. In the process according to claim 1 the active 10 enzyme selected from the group consisting of catalase, peroxidase, haemoglobin, and haenium.

## References Cited

## UNITED STATES PATENTS

3,062,650 11/1962 Sagura et al. ----- 96-90  
3,171,744 3/1965 Peticolas ----- 96-48 X

NORMAN G. TORCHIN, Primary Examiner

W. H. LOUIE, JR., Assistant Examiner

U.S. Cl. X.R.